

# UNITED STATES PATENT OFFICE.

PAUL C. SEEL, OF ROCHESTER, NEW YORK, ASSIGNOR TO EASTMAN KODAK COMPANY,  
OF ROCHESTER, NEW YORK, A CORPORATION OF NEW YORK.

## CELLULOSE-NITRATE COMPOSITION.

1,879,596.

Specification of Letters Patent.

Patented May 24, 1921.

No Drawing.

Application filed April 26, 1919. Serial No. 292,998.

To all whom it may concern:

Be it known that I, PAUL C. SEEL, a citizen of the United States of America, residing at Rochester, in the county of Monroe 5 and State of New York, have invented certain new and useful Improvements in Cellulose-Nitrate Compositions, of which the following is a full, clear, and exact specification.

10 This invention relates to a cellulose nitrate composition in which the cellulose nitrate is combined or mixed with other substances so that the resulting product can be advantageously used in such arts as sheet 15 or photographic film manufacture and varnish manufacture.

One object of my invention is to provide 20 a composition of matter, the inflammability of which is reduced to an important extent, so that it becomes relatively safe in use. Another object is to provide a composition which may be made into permanently transparent strong and flexible sheets or films 25 of desired thinness, that are substantially waterproof, are unaffected by ordinary photographic fluids and possess the desired properties of a support for sensitive photographic coatings. Another object of my invention is to produce a composition of 30 matter capable of easy manipulation in the film or varnish making and allied arts; which will not injure or be injured by the machinery or substances with which it is associated during manufacture, storage, or 35 use. Further objects will hereinafter appear.

I have discovered that a composition of matter having the desirable qualities enumerated hereinabove can be obtained by 40 mixing or compounding cellulose nitrate with the monohydroxy aliphatic alcohols having more than two carbon atoms, such as fusel oil, butyl alcohol, amyl alcohol, etc., together with triphenyl phosphate. This 45 compounding is best performed by mixing the cellulose nitrate, the higher alcohol or alcohols, and the triphenyl phosphate with a solvent common to all of them, such as methyl alcohol, or acetone, or a mixture 50 thereof.

In carrying out one illustration of my invention, I employ from 175 to 400 parts (say for instance 250 parts) of methyl alcohol or acetone, or a mixture of these two 55 substances in any proportion relative to

each other. In such solvent I incorporate 50 parts of cellulose nitrate, such as nitrated cotton, 10 to 60 parts of fusel oil (say for instance 20 parts) and 5 to 50 parts of triphenyl phosphate (say for example 7.5 60 parts). The ingredients are mixed to form a homogeneous solution or flowable mass which is filtered if desired, such operation being generally employed if the mass is to be used for making transparent photo- 65 graphic film base. The fusel oil, triphenyl phosphate, methyl alcohol and acetone may be of commercial purity, being preferably in a condition which will not impart any serious amount of color to the resulting 70 film.

The above solution or mass is sufficiently thick and viscous to be properly flowed during the manufacture of film base, the methyl alcohol or acetone, or mixture thereof, volatilizing, but the mixture being such that the volatile solvent does not go off so rapidly as to impair the product. The resulting 75 films containing the unvolatilized ingredients are so flexible, smooth, transparent and 80 uniform that they may be used for any usual or preferred purpose. Due to their reduced inflammability they form excellent motion picture film support or base. They are practically waterproof and unaffected by ordinary photographic chemicals. The triphenyl 85 phosphate and the fusel oil, particularly the former, are of such low volatility that the amount lost during the desired life of the film is negligible and will not render 90 such film unserviceable. The triphenyl phosphate seems to impart a degree of suppleness to the film, as does also the fusel oil in a useful degree, and these substances moreover retain the clearness or transparency 95 of the film. The triphenyl phosphate is practically non-inflammable and the film containing it in the preferred proportions has its inflammability diminished to a very noteworthy and desirable extent. The tri- 100 phenyl phosphate does not during manufacture decompose or chemically re-act with or injure the other bodies associated with it in the solution, nor does it attack the metal parts of the machinery to any harmful degree.

Having thus described my invention, what I claim as new and desire to secure by Letters Patent is:

1. A viscous flowable composition of mat- 110

ter for forming tough, transparent, flexible sheets, comprising cellulose nitrate 50 parts, triphenyl phosphate 5 to 50 parts, a mono-hydroxy aliphatic alcohol having from four 5 to five carbon atoms 10 to 60 parts and a volatile solvent containing methyl alcohol 175 to 400 parts.

2. A viscous flowable composition of matter for forming tough, transparent, flexible 10 films, comprising cellulose nitrate 50 parts, triphenyl phosphate 5 to 50 parts, fusel oil 10 to 60 parts, and a mixture of acetone and methyl alcohol 175 to 400 parts.

3. As an article of manufacture a flowed, strong, flexible, transparent, waterproof, <sup>15</sup> sheet of reduced inflammability, comprising cellulose nitrate, a monohydroxy aliphatic alcohol containing from four to five carbon atoms, and triphenyl phosphate.

4. A composition of matter comprising <sup>20</sup> cellulose nitrate, triphenyl phosphate and fusel oil.

Signed at Rochester, New York, this 22nd day of April, 1919.

PAUL C. SEEL.